

## UNITED STATES PATENT OFFICE

2,419,153

## LUBRICANT AND THE LIKE

John M. Musselman, South Euclid, and Herman P. Lankelma, Shaker Heights, Ohio, assignors to The Standard Oil Company, Cleveland, Ohio, a corporation of Ohio

No Drawing. Application April 9, 1943,  
Serial No. 482,491

14 Claims. (Cl. 252—32.7)

1

This invention relates to lubricants, and more particularly lubricants which are subject to severe usage conditions and in high temperature; and it is among the objects of the invention to provide lubricants having greater stability and resistance against change and having greater film strength than characteristic of usual petroleum lubricants.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

We have found that by reacting phosphorus pentasulphide with an organic oxygen-containing compound, products result which have peculiar utilities. The organic oxygen-containing compound employed is desirably of rather high molecular weight, and preferably of at least 300° F. boiling point, and involves esters, components thereof, ketones, and amino or halogen derivatives of these. The esters are alkyl or cycloparaffin or aryl esters of the organic acids. Illustrative of some conveniently applicable materials are: octyl laurate, butyl stearate, ethyl lactate, methyl oleate, butyl ricinoleate, dibutyl phthalate, methyl stearate, methyl dichlorostearate, methyl chloronaphthalene, dichloropalmitic acid, sperm oil, degras, beeswax, lanolin, and other waxes, cocoanut oil, other fatty oils, ethylene glycol mono ethers, diglycol chlorhydrin, isophorone, stearic acid, oleic acid, palmitic acid, myristic acid, naphthalic acid, benzoic acid, naphthoic acids, naphthenic acids, hydroxy stearate acids, dihydroxy benzoic acids, hydroxy naphthenic acids, dihydroxy stearic acids, chloro benzoic acids, dichloro stearic acids, oxidized petroleum fatty acids, lactones, oxidized oil, dichloro benzoic acid, dichloro dihydroxy stearic acid, etc.

On heating the organic compound and the phosphorus sulphide a reaction sets in at rather low temperatures, and a product of the general phosphoric acid type containing both phosphorus and sulphur is formed. For most compounds this occurs up to around 200° F., but for fatty oils it may extend to around 325° F. At higher temperatures however, there is a different type of reaction, and thiophosphoric compounds are decomposed, and phosphorus is eliminated as oxide. Preferably, we conduct reaction at such higher

2

range of temperature, as for instance 340° to around 400° F., or at least such as to involve the type of reaction above phosphate formation, and resulting in compounds in which higher percentages of sulphur are combined, and usually not over a half of one per cent of phosphorus, phosphorus being thrown out as oxide in sludge. Usually a reaction time of a half to an hour or somewhat more is sufficient. The materials may be taken in calculated or molecular proportions, however, a final excess of phosphorus pentasulphide may be easily eliminated by filtering off. For example thus, 300 parts of dichlorostearic acid may be reacted with 110 parts of phosphorus pentasulphide for 60 minutes.

With particular further advantage, the reaction product as foregoing, may be further reacted, or at least partially neutralized, with a base, which may be an amine, ammonia or oxides or hydroxides of metals, for example aluminum, lead, tin, calcium, barium, sodium, potassium, etc. This reaction occurs readily at temperatures in the range of 70° F. to 200° F.

The reaction products may be employed as such in certain usages, as for instance gear lubrication, or they may be incorporated in an oil of lubricating viscosity, as for instance in oils of 40 to 3000 viscosity Saybolt Universal at 100° F., and the amounts may be for instance 0.05-10 per cent.

This application is a continuation, in part, and as to common subject matter, of our application Serial No. 397,178, filed September 29, 1939, now issued as Patent No. 2,361,957 of November 7, 1944.

Other modes of applying the principle of the invention may be employed, change being made as regards the details described, provided the features stated in any of the following claims, or the equivalent of such, be employed.

We therefore particularly point out and distinctly claim as our invention:

1. In a process of preparing lubricants, reacting an unpolymerized organic oxygen-containing compound forming oil-soluble metal phosphorus sulfide reaction products and having a boiling point not less than 300° F. with phosphorus pentasulphide at a temperature above phosphate formation, and converting the product into a barium compound.

2. In a process of preparing lubricants, reacting an unpolymerized organic oxygen-containing compound forming oil-soluble metal phosphorus sulfide reaction products and having a boiling point not less than 300° F. with phosphorus

pentasulphide at a temperature above phosphate formation, and converting the product into a calcium compound.

3. In a process of preparing lubricants, reacting an unpolymerized organic oxygen-containing compound forming oil-soluble metal phosphorus sulfide reaction products and having a boiling point not less than 300° F. with phosphorus pentasulphide at a temperature above phosphate formation, and converting the product into an 10 aluminum compound.

4. In a process of preparing lubricants, reacting an unpolymerized organic oxygen-containing compound forming oil-soluble metal phosphorus sulfide reaction products and having a boiling point not less than 300° F. with phosphorus pentasulphide at a temperature above phosphate formation, and converting the product into a 15 metal compound.

5. In a process of preparing lubricants, reacting an unpolymerized organic oxygen-containing compound forming oil-soluble metal phosphorus sulfide reaction products and having a boiling point not less than 300° F. with phosphorus pentasulphide, and converting the product into a 20 metal compound.

6. In a process of preparing lubricants, reacting an unpolymerized aliphatic oxygen-containing compound forming oil-soluble phosphorus sulphide reaction products and having a boiling 25 point of not less than 300° F. with phosphorus pentasulphide at a temperature above phosphate formation.

7. In a process of preparing lubricants, mixing an unpolymerized aliphatic oxygen-containing compound forming oil-soluble phosphorus sulphide reaction products and having a boiling point of not less than 300° F. with phosphorus pentasulphide, and reacting said compound with said sulphide at a temperature above phosphate formation, said compound and said sulphide being mixed in calculated proportions to form a reaction product and a phosphorus-containing sludge at said reaction temperature, and separating the reaction product from the sludge. 30

8. A lubricant comprising the product of reaction of an unpolymerized organic oxygen-containing compound forming oil-soluble metal phosphorus sulfide reaction products and having a boiling point not less than 300° F. with phosphorus pentasulphide at a temperature above phosphate formation, and in turn converted into a barium compound.

9. A lubricant comprising the product of reaction of an unpolymerized organic oxygen-containing compound forming oil-soluble metal phosphorus sulphide reaction products and having a boiling point not less than 300° F. with phosphorus pentasulphide at a temperature above 35

4  
phosphate formation, and in turn converted into a calcium compound.

10. A lubricant comprising the product of reaction of an unpolymerized organic oxygen-containing compound forming oil-soluble metal phosphorus sulphide reaction products and having a boiling point not less than 300° F. with phosphorus pentasulphide at a temperature above phosphate formation, and in turn converted into an aluminum compound.

11. A lubricant comprising the product of reaction of an unpolymerized organic oxygen-containing compound forming oil-soluble metal phosphorus sulphide reaction products and having a boiling point not less than 300° F. with phosphorus pentasulphide at a temperature above phosphate formation, and in turn converted into a metal compound.

12. A lubricant comprising the product of reaction of an unpolymerized organic oxygen-containing compound forming oil-soluble metal phosphorus sulphide reaction products and having a boiling point not less than 300° F. with phosphorus pentasulphide and converted in turn to a metal compound.

13. A lubricant comprising the product of reaction of an unpolymerized aliphatic oxygen-containing compound forming oil-soluble phosphorus sulphide reaction products having a boiling point of not less than 300° F. with phosphorus pentasulphide at a temperature above phosphate formation.

14. A lubricant comprising the product of reaction of an unpolymerized aliphatic oxygen-containing compound forming oil-soluble phosphorus sulphide reaction products having a boiling point of not less than 300° F. with phosphorus pentasulphide at a temperature above phosphate formation and in calculated proportions to form a phosphorus-containing sludge separable from said reaction product.

JOHN M. MUSSelman.  
HERMAN P. LANKELMA.

#### REFERENCES CITED

The following references are of record in the file of this patent:

#### UNITED STATES PATENTS

| Number    | Name                    | Date          |
|-----------|-------------------------|---------------|
| 2,316,085 | Kelso et al. -----      | Apr. 6, 1943  |
| 2,242,260 | Prutton -----           | May 20, 1941  |
| 2,142,998 | Chittick -----          | Jan. 10, 1939 |
| 2,167,867 | Benning -----           | Aug. 1, 1939  |
| 2,331,923 | Musselman -----         | Oct. 19, 1943 |
| 2,252,985 | Rutherford et al. ----- | Aug. 19, 1941 |
| 2,252,984 | Rutherford et al. ----- | Aug. 19, 1941 |
| 2,169,634 | Cantrell et al. -----   | Aug. 15, 1939 |